

## UNITED STATES PATENT OFFICE

2,150,341

## ALLOY STEEL

Byramji D. Saklatwalla, Pittsburgh, Pa.

No Drawing. Application March 12, 1937,  
Serial No. 130,515

## 3 Claims. (Cl. 75—125)

This invention relates to alloy steels and particularly to alloy steels containing a high silicon content combined with copper and phosphorus, and especially containing carbon in the lower ranges of carbon content of steels.

This application is a continuation in part of my applications Serial Nos. 50,928, filed November 21, 1935, and 701,231, filed December 6, 1933.

The main object of my invention is to produce by the use of very cheap alloying elements an alloy steel containing low amounts of alloying elements and possessing a corrosion resistance to mild corroding media, such as the atmosphere. Another object of my invention is to produce such steels of comparatively low carbon content obtaining the strength properties in the steel principally from the alloy content and thus obviating the lack of ductility and other deleterious properties which are introduced when strength is obtained in steels by merely increasing the carbon content.

Alloy steels resistant to corrosion are produced by the use of elements such as chromium, tungsten, cobalt, aluminum, titanium, nickel and the like, which are comparatively expensive, and require appreciable contents of such elements to be present in the steel to obtain corrosion resistance. Very many of the above enumerated elements have the further disadvantage that they are readily oxidizable in the processes of steel making and therefore a considerable loss of values occurs when the scrap containing such elements is remelted for the production of new steel.

Further, comparatively cheap alloy steels are produced by the introduction in the steel of copper, either alone or together with slight percentages of phosphorus. Such steels, in order to display any appreciable resistance, for instance to atmospheric corrosion, have to contain an appreciable amount of copper, even up to approximately 1%. Whether slight amounts of phosphorus are added to such copper steel or not, it is well known that such steel has the objectionable property of being very difficultly rolled, formed and fabricated. Such steels are especially objectionable where the steel in the processes of manufacturing has to be heated to a high temperature and allowed to cool. It is well known that when such appreciable percentages of copper are present in the steel, such steel is subject to precipitation hardening. When the amounts of copper are kept low, such, for instance, as found in the ordinary copper-bearing steels, namely, between .20% and .30%, whether phosphorus is

simultaneously present or not, such steels display a very low degree of corrosion resistance.

Silicon has been used as a corrosion-resisting element in steel generally in conjunction with another element such as chromium. If silicon is utilized alone for this purpose, the percentages required for bringing about corrosion resistance are so high as to cause the resultant steel to be hard, brittle and practically incapable of fabrication by the ordinary processes. Silicon is utilized in the manufacture of all steels as a deoxidizing agent and certain residual percentages of it are left in the steel as insurance of complete deoxidation. In other cases, as in silicon structural steels, a higher percentage is intentionally left or added to impart strength. In the ordinary steels the contents of residual silicon left from deoxidation vary from approximately .15% to .35%. When silicon is added as the strengthening alloying element, its content generally runs up higher than .35%, even up to 1%. Even with such silicon percentages the steel displays some degree of brittleness, coarse structure and decreased weldability compared to carbon steels of the same strength. Such steels, up to even 1% of silicon, however, do not possess any appreciable corrosion resisting properties. On the contrary, in some cases, depending upon the contents of the other elements, such as carbon, sulphur and manganese, etc., it has been claimed that such a silicon content, in fact, accelerates atmospheric corrosion.

By the composition of my invention I have obviated the above enumerated deficiencies. I have eliminated the high cost of expensive corrosion resistant elements. Further, I have brought about the corrosion resistance by the use of comparatively very small percentages of each of the alloying elements. This is an advantage as it is recognized that steels of low alloy content are more uniform and reliable in properties. By the combination of silicon and copper in the presence of phosphorus I bring about a considerable degree of corrosion resistance without going to the high percentages of silicon or of copper with their accompanying deleterious physical properties. Similarly I have been able to utilize the corrosion resisting properties of a fairly high phosphorus content without introducing the well known deleterious effects of phosphorus. I accomplish this by the combined use of silicon and copper in the right proportions, in conjunction with the phosphorus. I have also found that by maintaining the carbon percentages in the lower ranges of steel, namely, approx-

5

10

15

20

25

30

35

40

45

50

55

imately between .01% and .25%, I can produce silicon-copper-phosphorus steels, possessing ample strength as well as ductility, without the deleterious effects of a high carbon content such as propensity towards lack of impact strength or reduced ductility. Further, the combination of elements of my invention produces a steel which is readily weldable by the ordinary processes of welding.

10 I have found that by the proper combination of silicon with copper and phosphorus within certain limits of each of these elements, together with definite limits of the carbon content, very useful corrosion resistant steels suitable for general purposes can be obtained at a reasonable cost. I have found that, in order to obtain high tensile steels with a high degree of ductility and corrosion resistance, together with resistance to shock and a good degree of weldability, the elements silicon, copper, phosphorus and carbon are required to be within the following limits:

|               | Per cent     |
|---------------|--------------|
| Silicon       | 1.10 to 1.65 |
| Copper        | .15 to .60   |
| 25 Phosphorus | .10 to .22   |
| Carbon        | .01 to .25   |

While useful steels are obtained in the above ranges of elements, I have found that steels with particularly good strength and ductility, together with corrosion resistance, are obtained when the alloying elements and carbon are kept within the following ranges:

|            | Per cent     |
|------------|--------------|
| 35 Silicon | 1.20 to 1.35 |
| Copper     | .30 to .45   |
| Phosphorus | .12 to .15   |
| Carbon     | .07 to .12   |

40 Besides the property of resistance to corrosion from the atmosphere, and from other mild corroding media, I have found that my steels containing silicon, copper, and phosphorus are also resistant to the action of high temperatures and possess comparatively higher strength and resistance to scaling than carbon steels of equivalent strength properties. These useful properties at high temperature are derived without the use of expensive elements, such as chromium, tungsten and the like which are commonly incorporated in steels used at high temperatures.

45 For resistance to mild corrosion, such as the atmosphere, when copper alone is used it is found that the percentage required to bring about any appreciable resistance is somewhere in the neighborhood of about .75% to 1%. Such high percentages of copper are accompanied by appreciable deficiencies in the physical property of the steel. Steels containing such amounts of copper are difficult to roll and fabricate inasmuch as 50 the surface and edges of such rolled material are not good and appreciable hardening takes place if such steel is cooled from a high temperature. It is well known that when copper is present in such percentages, on cooling from a high temperature 55 the copper precipitates in a finely divided form and thus precipitation hardening of the steel sets in. The addition of phosphorus to the copper steel augments the corrosion resistance but does not materially offset the mechanical difficulties 60 encountered by the high copper content. Such percentages of copper raise the yield point of the steel but do not materially impart strength if the carbon content is low, such as between .06% and .12%. For producing the requisite strength, 65 therefore, the carbon content has to be appre-

ciably raised, which is an undesirable feature, as it is well known that the physical deficiencies of high copper content are accentuated by the presence of a high carbon content. Similarly, if corrosion resistance is to be derived from a silicon content alone, it will have to be comparatively high, for instance, in the neighborhood of between 3% and 5% to be effective. Further, in the presence of silicon alone, the non-corrosive properties of phosphorus cannot well be utilized 10 as the presence of phosphorus accentuates the brittleness due to silicon if some other offsetting element, such as copper, is not present.

I have found that when I combine silicon in the broader range given above, namely, between 15 1.10% and 1.65%, with a copper range of .15% to .60% and phosphorus from .10% to .22% I can bring about corrosion resisting properties in such steel without showing the deficiencies either of a high copper or of a high silicon content. I, 20 further, achieve a corrosion resistance in the steel much greater than would be obtained by, say, 1% copper alone or together with phosphorus or by, say, 3% silicon. At the same time I utilize the corrosion resistant properties of the 25 cheap element phosphorus offsetting its deleterious effects. I have found that I can introduce in this combination of silicon and copper a phosphorus content of between .10% and .20%, which is much higher than the phosphorus content 30 found in ordinary commercial steels. It is well known that when a steel contains a high percentage of phosphorus, such as the above, it becomes brittle and particularly so at low temperatures. I have found that in the presence of the 35 above combination of silicon and copper such deleterious properties due to phosphorus are not present but that the corrosion resistance of the silicon-copper combination is very considerably increased by the phosphorus content. I have 40 further found that the phosphorus helps to augment the useful strength of the steels and therefore enables such steels to be produced with very low carbon contents comparatively to their strength.

I have found that strength is obtained in the steels of my above combination with comparatively low carbon contents. This is a great advantage particularly in steels which contain silicon, copper, and phosphorus. It is well known that when silicon, copper or phosphorus are present individually in steel that the higher the carbon content of such steel the more pronounced are the deleterious properties due to these elements. While such deleterious properties of the 55 individual elements are offset by a proper balancing of the elements in my combination, the deleterious properties of each of the elements being suppressed by the presence of the one or combination of two of the other elements, nevertheless 60 it is advantageous, to keep low the presence of an element like carbon which is known to produce deleterious effects in the presence of the individual elements.

A further advantageous feature of my invention is the fact that in counteracting the brittleness due to the high silicon content I use an element such as copper, which augments at the same time the corrosion-resistant property of the silicon. Further the combination of silicon and copper counteracts the deleterious properties of the phosphorus at the same time taking advantage of its corrosion and heat resisting properties. The combination, therefore, permits the full play 70 of the corrosion resistant and the heat resistant 75

properties of the individual elements, at the same time suppressing the deleterious physical properties which would be brought about by the individual elements if they were not present in this combination and in the ranges given. Further, this new composition of my steels has the added advantage that the elements used are all obtainable at a very cheap cost and are elements which are available and used in any ordinary steel making operation.

In the composition of my steel, besides the good physical properties, the corrosion resistance is brought about by the balanced percentages of the elements, silicon, copper, phosphorus, without the necessity of addition of other expensive elements, such as nickel, tungsten, titanium, vanadium, zirconium, aluminum and the like. Such elements, however, can be present in small amounts, to fractions of a percent, without affecting the properties of my steel. Manganese and sulphur may be present in the amounts usually found in common steels, although I prefer to have not over about .5% manganese and not over about .05% sulphur.

The steels of my invention can be manufactured by the ordinary steel making processes, such as the Bessemer, open hearth, crucible or electric furnace process. The silicon content can be introduced in the usual manner by the use of ferro-silicon of the percentages commonly available in commerce. The ferro-silicon may be added in the furnace, but it is desirable to add some in the form of a high percentage ferro-silicon, such as 75% or 90%, in the ladle in order to obtain a more accurate final content of silicon in the steel. The copper may be added in the furnace, and small additions for final correction of the analysis may be made in the ladle. The phosphorus may be added in the form of ferro-phosphorus or may be partly derived from the phosphorus content of some of the ingredients used in melting and refining the steel. Part of the ferro-phosphorus may be added in the furnace and then the rest added in the ladle to obtain more definite control of the analysis of the finished steel. Owing to the rapid oxidizability of

phosphorus it is recommendable to add the main bulk, if not all, of the ferro-phosphorus in the ladle. In the casting, rolling and other fabricating operations of the steel the behavior of my composition is not any different to that of usual steels of equal physical properties.

The steels of my composition possess the physical properties of strength, ductility, weldability, etc., in the as-rolled condition, but they are capable of heat treatment to develop and produce necessary different properties in particular cases. The steels of my composition are capable of being produced in the forms of all the ordinary products usually produced by steel works. They can be fabricated into billets, slabs, bars, rods, plates, shapes, sheets, tubes, wire and the like.

While I have specifically described the preferred embodiment of my invention, the invention may be otherwise embodied and practiced within the scope of the following claims.

I claim:

1. A steel of low carbon content between .01 and .25% carbon, containing as essential alloying constituents 1.10% to 1.65% silicon, .15 to .60% copper and .10 to .22% phosphorus not over about .5% manganese and not over about .05% sulphur, the balance being substantially all iron, and characterized by corrosion resistance, strength, ductility and weldability.

2. A steel of low carbon content between .07 and .12% carbon, containing as essential alloying constituents 1.20 to 1.35% silicon, .30 to .45% copper, .12 to .15% phosphorus, not over about .5% manganese and not over about .05% sulphur, the balance being substantially all iron, and characterized by corrosion resistance, strength, ductility and weldability.

3. A steel of low carbon content between .01 and .25% carbon, containing as essential alloying constituents 1.20-1.65% silicon, .15-.60% copper, .10-.22% phosphorus not over about .5% manganese and not over about .05% sulphur, the balance being substantially all iron, and characterized by corrosion resistance, strength, ductility and weldability.

BYRAMJI D. SAKLATWALLA.